# EUROPEAN PATENT SPECIFICATION

(11) **EP 3 075 904 B1**
(45) Date of publication and mention of the grant of the patent: **08.11.2017**
(21) Application number: 15161983.0
(22) Date of filing: 31.03.2015
(51) Int. Cl.: D21H 19/38, B65D 65/42, D21H 19/56, D21H 19/58

(54) **SUBSTRATE WITH STRETCHABLE COATING**
SUBSTRAT MIT DEHNBARER BESCHICHTUNG
SUBSTRAT AVEC REVÊTEMENT ÉTIRABLE

(43) Date of publication of application: 05.10.2016
(73) Proprietor: BillerudKorsnäs AB, 169 27 Solna (SE)
(72) Inventor: Larsson, Mikael, SE-656 37 Karlstad (SE); Ragnarsson, Micael, SE-660 50 Vålberg (SE); Kritzinger, Johannes, CH-4600 Olten (CH); Schölkopf, Joachim, CH-8956 Killwangen (CH)
(74) Representative: Kransell & Wennborg KB

(56) References cited:
- WO-A1-2008/122617
- WO-A1-2010/114467
- US-B1- 6 740 373

## Description

### TECHNICAL FIELD

The invention relates to a paper substrate provided with a stretchable coating.

### BACKGROUND

Pigment coatings are widely used to enhance optical properties, such as gloss and print quality, of paper and paperboard. Pigment coatings may also improve other properties of a paper or paperboard product.

### SUMMARY

The present inventors have observed an impaired visual impression of the print on pigment-coated paper products after the paper products have been stretched. The inventors have realized that the problem is caused by cracks formed in the pigment coating layer during stretching.

The stretching in question may for example occur when a sheet of the paper product is given a three-dimensional shape in a press-forming or thermo-forming operation. Further, the stretching may occur when the paper product is bended or folded, e.g. to form a package.

Accordingly, the present inventors have realized that there is a need for a paper substrate provided with a "stretchable coating", i.e. a coating that does not crack to such an extent that the visual impression of a print on the coating is significantly impaired when the paper substrate is stretched.

The following itemized listing of embodiments of the present disclosure is presented to meet the above-mentioned need.
1. A coated paper material comprising a paper substrate coated with a composition comprising:
   at least one polymeric binder having a glass transition temperature (Tg) of -3 °C or lower, and
   at least one inorganic filler having a BET specific surface area in the range of 2.0 to 20.0 m²/g,
   wherein the dry weight ratio of the at least one polymeric binder to the at least one inorganic filler is between 15:100 and 20:100, such as between 16:100 and 20:100 and
   wherein the at least one polymeric binder is at least one acrylic binder and wherein the coated paper material according to any one of the preceding items, wherein the at least one polymeric binder and the at least one inorganic filler together constitute at least 90 wt.-% of the composition, based on the dry weight of the composition..
2. The coated paper material according to item 1, wherein the paper substrate comprises at least two paper layers including a top paper layer that is coated with the composition.
3. The coated paper material according to item 1 or 2, wherein the stretchability (ISO 1924/3) of the paper substrate or the top paper layer thereof is at least 3 % in the machine direction (MD) and/or the cross direction (CD).
4. The coated paper material according to item 3, wherein the stretchability (ISO 1924/3) of the paper substrate or a top paper layer thereof is at least 5 % in the machine direction (MD) and/or the cross direction (CD).
5. The coated paper material according to item 4, wherein the stretchability (ISO 1924/3) of the paper substrate or a top paper layer thereof is at least 7 % in the machine direction (MD) and/or the cross direction (CD).
6. The coated paper material according to any one of the preceding items, wherein the stretchability (ISO 1924/3) of the paper substrate or a top paper layer thereof is at least 12 % in the machine direction (MD).
7. The coated paper material according to any one of the preceding items, wherein the Tg of the at least one polymeric binder is -10 °C or lower, such as -15 °C or lower, such as -20 °C or lower.
8. The coated paper material according to any one of the preceding items, wherein the BET specific surface area of the at least one inorganic filler is in the range of 3.0 to 17.5 m²/g, such as 4.0 to 15 m²/g, such as 5.0 to 13 m2/g.
9. The coated paper material according to any one of the preceding items, wherein the at least one polymeric binder is selected from the group consisting of:
   acrylic homopolymers;
   methacrylic homopolymers;
   copolymers composed of at least two different monomers, one monomer having an acrylic or methacrylic functional group and the other monomer having a functional group selected from the group consisting of styrene, vinyl and allyl; and
   mixtures thereof.
10. The coated paper material according to any one of the preceding items, wherein the at least one polymeric binder is an acrylic homopolymer, a vinyl-acrylic copolymer, a styrene-acrylic copolymer, or a mixture thereof.
11. The coated paper material according to any one of the preceding items, wherein the weight median particle size *d₅₀* of the at least one inorganic filler is in the range of 0.1 to 5.0 µm, such as 0.3 to 3.0 µm, such as 0.4 to 2.0 µm, such as 0.5 to 1.5 µm.
12. The coated paper material according to any one of the preceding items, wherein the weight median particle size *d₉₈* of the at least one inorganic filler is in the range of 1.0 to 20.0 µm, such as 2.0 to 12.0 µm, such as 3.0 to 6.0 µm.
13. The coated paper material according to any one of the preceding items, wherein the at least one inorganic filler is selected from the group consisting of calcium carbonate containing material, talc, kaolin, clay, titanium dioxide, satin white, bentonite and mixtures thereof.
14. The coated paper material according to item 13, wherein the at least one inorganic filler is selected from the group consisting of calcium carbonate containing material, clay, kaolin and mixtures thereof.
15. The coated paper material according to item 14, wherein the at least one inorganic filler is a calcium carbonate containing material.
16. The coated paper material according to item 15, wherein calcium carbonate containing material is selected from the group consisting of natural ground calcium carbonate (GCC), precipitated calcium carbonate (PCC), dolomite and mixtures thereof.
17. The coated paper material according to item 16, wherein calcium carbonate containing material is natural ground calcium carbonate selected from the group consisting of marble, limestone, chalk and mixtures thereof.
18. The coated paper material according to item 16, wherein calcium carbonate containing material is precipitated calcium carbonate selected from the group consisting of rhombohedral PCC (R-PCC), scalenohedral PCC (S-PCC) and aragonitic PCC (A-PCC).
19. The coated paper material according to any one of the preceding items, wherein the at least one polymeric binder and the at least one inorganic filler together constitute at least 90 wt.-% of the composition, based on the dry weight of the composition.
20. The coated paper material according to any one of the preceding items, wherein the composition comprises at least one further additive selected from the group consisting of thickeners, lubricants, dispersants, milling aids, rheology modifiers, defoamers, optical brighteners, dyes, pH controlling agents and mixtures thereof.
21. The coated paper material according to any one of the preceding items, wherein the at least one inorganic filler constitutes 75 to 88 wt.-% of the composition, based on the dry weight of the composition.
22. The coated paper material according to any one of the preceding items, wherein the at least one polymeric binder constitutes 12 to 17 wt.-% of the composition, based on the dry weight of the composition.
23. The coated paper material according to any one of the preceding items, wherein the at least one further additive constitutes 0.1 to 8 wt.-% of the composition, based on the dry weight of the composition.
24. The coated paper material according to any one of the preceding items, wherein the paper substrate or at least a layer thereof is composed of Kraft paper.
25. The coated paper material according to any one of the preceding items, wherein a coated surface of the coated paper material is printed.
26. The coated paper material according to item 25, wherein the printed surface is covered by a barrier layer.
27. The coated paper material according to any one of items 1-24, wherein a coated surface is covered by a barrier layer.
28. A blank provided with folding lines, which blank is composed of the coated paper material according to any one of the preceding items.
29. A package comprising at least one wall composed of the coated paper material according to any one of items 1-27.
30. A package comprising at least two walls composed of the coated paper material according to any one of items 1-27, which walls are joined by an edge defined by a folding line formed in the coated paper material.
31. A box comprising a bottom wall and at least two side walls composed of the coated paper material according to any one of items 1-27.
32. The coated paper material, blank, package or box according to any one of the preceding items comprising a bulge or relief formed by stretching a portion of the coated paper material.
38. A method of forming a three-dimensional pattern comprising a step of subjecting an article comprising a coated paper material according to any one of items 1-27 to a forming operation, such as press-forming or thermo-forming, to form the three-dimensional pattern in the coated paper material, wherein part of the coated paper material is stretched during the forming operation.

### BRIEF DESCRIPTION OF THE DRAWINGS

The invention is now described, by way of example, with reference to the accompanying drawings, in which:
Figs 1a-1d illustrate different embodiments of a coated paper material according to the present disclosure.
Fig 2 illustrates a blister pack composed of a coated paper material according to the present disclosure that has been stretched in a forming operation.
Figs 3 and 4 illustrate trays composed of a coated paper material according to the present disclosure that has been stretched in a forming operation.
Fig 5 illustrates a clamshell package composed of a coated paper material according to the present disclosure that has been stretched in a forming operation.
Fig 6 illustrates a base portion of another clamshell package. The vase portion is composed of a coated paper material according to the present disclosure that has been stretched in a forming operation.
Fig 7 illustrates a sleeve 700 composed of a coated paper material according to the present disclosure. Part of the sleeve has been stretched in a forming operation such that a decorative/descriptive relief text is obtained.
Fig 8 illustrates a box for a wine bottle composed of a coated paper material according to the present disclosure. Part of the coated paper material has been stretched in a forming operation such that a decorative/descriptive relief in the shape of a wine bottle is obtained has been formed in a side wall of the box.
Fig 9a - d show a diagonal top view (fig. 1a), side view (fig. 1b), top view (fig. 1c) and front view (fig. 1d) of a 3D formability tester.

### DETAILED DESCRIPTION

As a first aspect of the present disclosure, there is thus provided a coated paper material comprising a paper substrate coated with a composition.

The paper substrate may for example comprise at least two paper layers. In such case, the substrate will have a top paper layer and a bottom paper layer. Further, the top paper layer will be coated with the composition. Optionally, the bottom paper layer is also coated with the composition. This means that the top surface of the paper substrate is covered by the coating composition and the bottom surface of the paper substrate is optionally covered by the coating composition.

The coat weight of each coating layer may for example be 4-40 g/m², such as 5-35 g/m², such as 5-30 g/m², such as 8-25 g/m², such as 15-25 g/m². If the coat weight is too low, there is a great risk that areas of insufficient coverage is obtained. A coating layer may comprise two or more sublayers

The paper substrate may for example be a laminate, in which at least two paper layers are adhered to each other. The adhesive may for example be a layer of polyethylene (PE), a water-based glue or an organic solvent-based glue. The amount of adhesive provided between two layers in the paper substrate may for example be 2-35 g/m², such as 4-20 g/m².

The grammage of the paper substrate may for example be 40-550 g/m², such as 75-550 g/m². When the paper substrate comprises a single paper layer, the grammage of the paper substrate may for example be 40-200 g/m², such as 50-150 g/m² or 75-200 g/m². When the paper substrate comprises at least two paper layers, the grammage of the paper substrate may for example be 80-550 g/m², such as 100-550 g/m², such as 150-500 g/m². When the paper substrate comprises at least three paper layers, the grammage of the paper substrate may for example be 175-550 g/m², such as 250-550 g/m², such as 300-550 g/m².

In embodiments of the first aspect, the stretchability (ISO 1924/3) of the paper substrate is at least 3 % in the machine direction (MD) and/or the cross direction (CD). In preferred embodiments, the stretchability (ISO 1924/3) of the paper substrate is at least 5 or 7 % in the machine direction (MD) and/or the cross direction (CD). In one embodiment, the stretchability (ISO 1924/3) of the paper substrate is at least 12 % or 14 % in the machine direction (MD).

An example of a suitable material for the paper substrate is FibreForm® marketed by BillerudKorsnäs AB (Sweden). In FibreForm®, the stretchability is at least 7 % in the CD and at least 13 % in the MD.

In the embodiments wherein the paper substrate comprises more than one layer, the stretchability (ISO 1924/3) of top layer may be at least 3, 5, 7, 12 or 14 % in the machine direction (MD) and/or the cross direction (CD). In such embodiments, the stretchability (ISO 1924/3) of at least one other layer may be below 5 or 3 % in the machine direction (MD) and/or the cross direction (CD).

It is understood from the discussion above that the benefits of the stretchability of the coating of the present disclosure is more relevant when the stretchability of the paper substrate (or at least the top layer thereof) is higher.

A paper substrate or paper layer of the present disclosure having a stretchability of at least 5 % in the machine direction (MD) and/or the cross direction (CD) is preferably at least partly obtained from chemical pulp, which generally has longer fibres than mechanical pulp. For example, the paper substrate or paper layer having such a stretchability may be composed of Kraft paper. In one embodiment, the paper substrate comprises more than one layer and at least the top layer is composed of Kraft paper.

The inventors have noted that the stretchability of the composition partly depends on the Tg of the polymeric binder. If the Tg is too high, the stretchability is insufficient. Accordingly, the composition of the present disclosure comprises at least one polymeric binder having a Tg of -3 °C or lower, preferably -10 °C or lower and more preferably -15 °C or lower. In one embodiment, the Tg is -20 °C or lower. A binder having a Tg of -25 °C has been shown to result in particularly beneficial coating properties.

If the Tg is too low, the coating may become too sensitive. Therefore, the Tg may be above -85 °C, such as above -70 °C, such as above -45 °C.

Preferred Tg ranges are -15 to -30 °C, such as -20 to -30 °C.

The glass transition temperature (Tg) is a well-known parameter to those skilled in the art, and is the temperature range, where a thermosetting polymer changes from a more pliable, compliant or "rubbery" state to a hard, rigid or "glassy" state upon cooling. The Tg is usually measured using Differential Scanning Calorimetry (DSC): ASTM E1356, "Standard Test Method for Assignment of the Glass Transition Temperature by Differential Scanning Calorimetry". The Tg is actually a temperature range, rather than a specific temperature. The convention, however, is to report a single temperature defined as the midpoint of the temperature range, bounded by the tangents to the two flat regions of the heat flow curve.

The polymeric binder of the present disclosure is an acrylic binder. Accordingly, the at least one polymeric binder is/are at least one acrylic binder.

In the context of the present disclosure, an "acrylic binder" refers to a polymeric binder comprising an acrylic monomer. Examples of acrylic monomers are methacrylates, methyl acrylate, ethyl acrylate, 2-ethylhexyl acrylate, hydroxyethyl methacrylate, butyl acrylate and butyl methacrylate.

The at least one polymeric binder is for example selected from the group consisting of: i) acrylic homopolymers; ii) methacrylic homopolymers iii) copolymers composed of at least two different monomers; and iv) mixtures thereof. "Mixtures thereof." refers to any mixture consisting of at least two of i)-iii).

In the copolymers of iii), one monomer has an acrylic or methacrylic functional group and the other monomer has a functional group selected from the group consisting of styrene, vinyl and allyl.

The at least one polymeric binder is preferably: a) an acrylic homopolymer; b) a vinyl-acrylic copolymer; c) a styrene-acrylic copolymer; or d) a mixture thereof. "Mixture thereof." refers to any mixture consisting of at least two of a)-c).

When the composition of the present disclosure is prepared, the polymeric binder is normally provided in the form of an aqueous dispersion. A specific example of a commercial aqueous dispersion of an acrylic homopolymer having a Tg of -30 °C is Appretan® E2100 (ARCHROMA). A specific example of a commercial aqueous dispersion of a styrene-acrylic copolymer having a Tg of -25 °C is Primal™ 325 GB (Dow). A specific example of a commercial aqueous dispersion of a styrene-acrylic copolymer having a Tg of -20 °C is Appretan® E6200 (ARCHROMA). A specific example of a commercial aqueous dispersion of a vinyl-acrylic copolymer having a Tg of -15 °C is Appretan® E4250 (ARCHROMA).

The composition of the present disclosure further comprises at least one inorganic filler. The presence of filler in the coating improves printability and other properties. The at least one inorganic filler may be selected from the group consisting of calcium carbonate containing material, talc, kaolin, clay, titanium dioxide, satin white, bentonite and mixtures thereof. "Mixtures thereof." refers to any mixture of at least two of the foregoing examples of inorganic fillers.

Calcium carbonate containing material, clay, kaolin or a mixture thereof are preferred examples.

When the inorganic filler is a calcium carbonate containing material, it is preferably selected from the group consisting of natural ground calcium carbonate (GCC), precipitated calcium carbonate (PCC), dolomite and mixtures thereof.

GCC is a particularly preferred example. The GCC may for example be selected from marble, limestone, chalk and mixtures thereof.

Another preferred example is PCC, which may be selected from rhombohedral PCC (R-PCC), scalenohedral PCC (S-PCC) and aragonitic PCC (A-PCC).

The BET specific surface area of the at least one inorganic filler is within the range of 2.0 to 20 m²/g. Preferred ranges are 3.0 to 17.5 m²/g, 4.0 to 15 m²/g and 5.0 to 13 m²/g. It has been found that if the specific surface area of the filler is too large (i.e. > 30 m²/g), cracks are easily formed in the coating. Without being bound by any specific scientific theory, the inventors believe that the average thickness of the binder films formed between the filler particles in the coating increases when the specific surface area of the filler decreases and that such an increase in thickness results in improved stretchability of the films and thus less crack formation.

The BET specific surface area is preferably measured with the analyzer Tristar II marketed by Micromeritics. Further, the measurement may be carried out according to the standard ISO 9277:1995.

It follows from the above that a relatively large filler particles are preferred as they result in a smaller specific surface area. Further, the inventors speculate that if fine particles are present in high amounts, they may form flakes that increase the crackability of the coating. Accordingly, the amount of very small filler particles is preferably kept low. However, if the filler particles are too large or coarse, the printing surface may become too rough, which may result in unsatisfactory gloss and/or brightness. As known to the skilled person, particle size distribution may be quantified by d values. For determining the weight median particle size d₅₀ value or the top cut particle size *d*₉₈ value a Sedigraph 5100 or 5120 device from the company Micromeritics, USA, can be used.

Preferably, the weight median particle size *d₅₀* of the at least one inorganic filler is in the range of 0.1 to 5.0 µm, such as 0.3 to 3.0 µm, such as 0.4 to 2.0 µm, such as 0.5 to 1.5 µm. Further, the weight median particle size *d₉₈* of the at least one inorganic filler is in the range of 1.0 to 20.0 µm, such as 2.0 to 12.0 µm, such as 3.0 to 6.0 µm.

Specific examples of a commercial GCC (marble) products having a BET specific surface area in the range of 1 to 30 m²/g are Hydrocarb® 60 - ME 78% (Omya), Hydrocarb® 90 - ME 78% (Omya) and Setacarb® HG - ME 75 % (Omya).

Hydrocarb ® 60 has a weight median particle size *d₅₀* of 1.4 µm and a weight median particle size *d₉₈* of 10 µm. Hydrocarb ® 90 has a weight median particle size *d₅₀* of 0.7 µm and a weight median particle size *d₉₈* of 5 µm. Setacarb® HG has a weight median particle size *d₅₀* of 0.5 µm and a weight median particle size *d₉₈* of 2 µm.

The inventors have found that another way of improving the stretchability of the coating is to have a relatively high ratio of the at least one polymeric binder to the at least one inorganic filler. The inventors believe that a relatively high ratio prevents crack formation as the film formed by the binder is less interrupted when the amount of filler is lower.

However, the ratio cannot be too high, because in such case the printability of the coating surface is insufficient. Further, the polymeric binder is generally more expensive than the inorganic filler and it is therefore beneficial to keep the ratio low from a cost perspective.

The inventors have identified a dry weight ratio of the at least one polymeric binder to the at least one inorganic filler in the range of 15:100 to 20:100 as an optimum when stretchability, printability and cost is taken into account.

Preferably, the ratio is in the range of 16:100 to 20:100.

In addition to the above-mentioned polymeric binder and inorganic filler, the composition of the present disclosure may at least one additive selected from the group consisting of:
thickeners (also referred as rheology modifiers), such as HASE rheology modifiers;
lubricants;
dispersants;
milling aids;
defoamers;
optical brighteners;
dyes; and
pH controlling agents.

As understood by the skilled person, the composition may also comprise a mixture consisting of two or more additives selected from the above.

However, the above-mentioned additives preferably constitute only a minor part of the composition, such as 0.1 to 8 wt.-% of the composition, based on the dry weight of the composition. The at least one polymeric binder and the at least one inorganic filler together constitute at least 90 wt.-% of the composition, based on the dry weight of the composition. In one embodiment, the at least one polymeric binder and the at least one inorganic filler together constitute at least 92 wt.-%, such as at least 92 wt.-%, of the composition, based on the dry weight of the composition.

It follows that the at least one inorganic filler for example constitutes 75 to 88 wt.-% of the composition, based on the dry weight of the composition.

It also follows that the at least one polymeric binder for example constitutes 12 to 17 wt.-% of the composition, based on the dry weight of the composition.

When the coated paper material of the present disclosure is prepared, the paper substrate may be composition may be applied as an aqueous coating composition having a solids content in the range of from 50 to 75 wt.-%, preferably in the range of 60 to 72 wt.-%, and most preferably in the range of 65 to 70 wt.-%, based on the total weight of the aqueous coating composition.

In the preparation of the aqueous coating composition, the components may, independently from each other, be provided in dry form, or in the form of suspensions, dispersions, slurries or solutions, and be mixed in any order. The mixing of the components may be carried out by any suitable mixing means known to those skilled in the art, for example a caddy mill. In one embodiment the aqueous coating composition may contain further solvents such as alcohol ethers, alcohols, aliphatic hydrocarbons, esters, and mixtures thereof.

The substrate may be coated, once or several times, with the aqueous coating composition, wherein the coating may be carried out by conventional techniques well-known in the art.

In embodiments of the present disclosure, a coated surface of the coated paper material is printed. Thus, a print comprising ink, such as flexographic ink, may be formed on the coated surface. Examples of flexographic inks are solvent-based inks, water-based inks, electron beam (EB) curing inks and ultraviolet (UV) curing inks. The print on the coated surface may thus be obtained by means of flexography.

The printed surface of the above-mentioned embodiments may covered by a barrier layer. Also, a coated surface of the coated paper material may be covered by a barrier layer, which means that the surface covered by the barrier layer is not printed.

The barrier layer has one or more barrier properties. Examples of barrier properties include grease barrier, gas barrier and moisture barrier properties. Such barrier properties are for example of interest when food or liquids are packaged.

The barrier layer may for example comprise or consist of PE (e.g. HDPE, LLDPE or LDPE), PLA, PA, PET, PP or Lacquer hot melt. Such barrier materials enable heat-sealing: Further, the barrier layer may be a dispersion, a bio-based polymer, a bio-based binding material or a glue. In one embodiment, the barrier layer comprises a platy clay, such as a hyperplaty clay, e.g. BARRISUR™ (Imerys).

A benefit of PE and PP is that they are moisture barriers.

The barrier layer may comprise sublayers. For example, it may comprise a layer of EVOH, which is a gas barrier, sandwiched between two layers of polyolefin, such as PE or PP. The barrier layer may also be a multilayer PA-polymer structure (PA is also a gas barrier).

A blank of the coated paper material of the present disclosure may be provided with folding lines, such that it may be folded into a three-dimensional object, such as a package (e.g. a box) or a part thereof (e.g. a lid).

It follows that a package may comprise at least one wall composed of the coated paper material of the present disclosure. In one embodiment of such a package, at least two walls are composed of the coated paper material according to the present disclosure, which walls are joined by an edge defined by a folding line formed in the coated paper material. A box may comprise a bottom wall and at least two side walls composed of the coated paper material of the present disclosure.

In a coated paper material, blank, package or box according to the present disclosure, a three-dimensional pattern, such as a bulge or relief, may be formed in the coated paper material. When such a three-dimensional pattern is formed, a portion of the coated paper-material is stretched.

As a second aspect of the present disclosure, there is provided a method of forming a three-dimensional pattern comprising a step of subjecting an article comprising a coated paper material of the present disclosure to a forming operation to form the three-dimensional pattern in the coated paper material. During the forming operation, part of the coated paper material is stretched. Hence, there is a benefit of using the stretchable coating of the present disclosure. The forming operation may for example be press-forming or thermo-forming.

### EXAMPLARY EMBODIMENTS

Fig 1a shows a non-limiting embodiment of a coated paper material 100 according to the present disclosure. The material 100 comprises a paper substrate 101 consisting of a single paper layer. The paper substrate 101 is preferably stretchable. For example, it may be composed of FibreForm® (BillerudKorsnäs AB, Sweden). The stretchability of FibreForm® is at least 7 % in the CD and at least 13 % in the MD when measured according to ISO 1924/3. The top surface of the paper substrate 101 is covered by a coating layer 102 consisting of a composition comprising an inorganic filler (e.g. calcium carbonate pigment) and an acrylic binder (e.g. styrene-acrylic copolymer). The coating layer 102 is printed such that a printing layer 103 is obtained. The printing layer 103 thus comprises ink. In turn, the printing layer 103 is covered by a barrier layer 104 having one or more barrier properties. Examples of barrier properties include grease barrier, gas barrier and moisture barrier properties. Such barrier properties are for example of interest when foods are packaged. The barrier layer 104 may have been applied to the printing layer by a coating method. Alternatively the barrier layer 104 may have been applied by gluing a plastic film to the printing layer. The barrier layer 104 may for example comprise two or more sublayers. For example, it may comprise a first and a second sub-layer consisting of PE and a third sub-layer, arranged between the first 111 and the second 112 sub-layer, consisting of EVOH. In such case, the PE layers mainly function as moisture barriers while the EVOH layer mainly functions as a gas barrier.

Fig 1b shows another non-limiting embodiment of a coated paper material 110 according to the present disclosure. The material 110 comprises a paper substrate 111 consisting of a single paper layer. As in the embodiment of Fig 1a, the paper substrate 111 is preferably stretchable and may be composed of FibreForm®. The top surface of the paper substrate 111 is covered by a coating layer 112a consisting of a composition comprising an inorganic filler (e.g. calcium carbonate pigment) and an acrylic binder (e.g. styrene-acrylic copolymer). Further, the bottom surface of the paper substrate 111 is covered by a coating layer 112b consisting of the same composition. The coating layers 112a, 112b are printed such that a top printing layer 113a and a bottom printing layer 113b are obtained. In turn, the printing layers 113a, 113b are covered by top and bottom barrier layers 104a, 104b having one or more barrier properties. Barrier layers and their properties are discussed above in connection with Fig 1a. The barrier properties of the top barrier layer 114a and the barrier properties of the bottom barrier layer 114b are not necessarily the same. For example, the top barrier layer 114a may comprise three sublayers as described above in connection with Fig 1a and thus have moisture and gas barrier properties, wile the bottom barrier layer consists of PE and mainly functions as a moisture barrier.

Fig 1c shows another non-limiting embodiment of a coated paper material 120 according to the present disclosure. The material 120 comprises a paper substrate 121 that is a laminate comprising a first (top) 121a and a second (bottom) 121b paper layer. Between the first 121a and the second 121b paper layer, a polyethylene (PE) layer 121c is provided as an adhesive. The amount of PE may for example be 20-30 g/m². The first 121a and the second 121b paper layers are stretchable and preferably composed of FibreForm®. Accordingly, the whole paper substrate 121 is stretchable. The top surface of the first (top) paper layer 121a is covered by a coating layer 122 consisting of a composition comprising an inorganic filler (e.g. calcium carbonate pigment) and an acrylic binder (e.g. styrene-acrylic copolymer). The coating layer 122 is printed such that a printing layer 123 is obtained. In turn, the printing layer 123 is covered by a barrier layer 124 having one or more barrier properties. Barrier layers and their properties are discussed above in connection with Fig 1a.

Fig 1d shows another non-limiting embodiment of a coated paper material 130 according to the present disclosure. The material 130 comprises a paper substrate 131 that is a laminate comprising a first (top) paper layer 131a, a second (middle) paper layer 131b, and a third (bottom) paper layer 131d. The second paper layer 131b is thus sandwiched between the first 131a and the third 131d paper layer. Between the paper layers 131a, 131b, 131d, polyethylene (PE) layers 131c, 131e are provided as adhesive. The amount of PE in each PE layer may for example be 20-30 g/m². The first 131a and the third 131d paper layers are highly stretchable and preferably composed of FibreForm®. The second paper layer 131b is however significantly less stretchable than FibreForm® and may be for example be formed from pulp comprising mechanical pulp, thermomechanical pulp (TMP) and/or chemithermomechanical pulp (CTMP). Accordingly, the whole paper substrate 131 is not highly stretchable, but the outer paper layers 131a and 131d are. The top surface of the first (top) paper layer 131a is covered by a coating layer 132 consisting of a composition comprising an inorganic filler (e.g. calcium carbonate pigment) and an acrylic binder (e.g. styrene-acrylic copolymer). The coating layer 132 is printed such that a printing layer 133 is obtained. In turn, the printing layer 133 is covered by a barrier layer 134 having one or more barrier properties. Barrier layers and their properties are discussed above in connection with Fig 1a.

Fig 2 shows a blister pack 200 formed in a coated paper material according to the present disclosure. A coated side is printed. The print is preferably covered by a barrier layer providing protection against gas and moisture (and possibly grease). The paper substrate of the material is composed of FibreForm®. The stretchability of the paper substrate and the coating enables the formation of a plurality of cavities 201 in the blister pack 200, e.g. by press-forming, thermo-forming or vacuum-forming, without significant impairment of the visual impression of the print. The underside of the cavities 201 appear as bulges 202 on the backside of the blister pack 200.

The blister pack 200 may for example be designed to contain pills (such as medical pills) or candy. It is understood that the cavities 201 of the blister pack 200 may be covered by a film or foil composed of plastic or aluminium, which film or foil is broken to obtain the contents of the blister pack 200. The grammage of coated paper material of the blister pack may for example be 150-300 g/m².

Fig 3 shows a rectangular tray 300 with rounded corners formed in a coated paper material according to the present disclosure. The paper substrate is composed of FibreForm®. A coated side of the material is printed. If the tray 300 is intended for foodstuffs, the coated paper material preferably comprises one or more barriers against gas and moisture and possibly grease. The stretchability of the substrate and the coating enables the formation of a body portion 301 and a circumferential rim portion 302 without significant impairment of the visual impression of the print. The body portion 301 comprises side walls and a bottom wall. The outer edge 303 of the rim portion 302 is bent downwards for increased stability and improved aesthetics. The tray 300 may be formed by press-forming, thermo-forming or vacuum-forming.

Fig 4 shows another embodiment of a tray 400, which is not rectangular, formed in a coated paper material according to the present disclosure. The paper substrate is composed of FibreForm®. A coated side of the material is printed. If the tray 400 is intended for foodstuffs, the coated paper material preferably comprises one or more barriers against gas and moisture and possibly grease. The stretchability of the paper substrate and the coating enables the formation of a body portion 401 and a flat circumferential rim portion 402 without significant impairment of the visual impression of the print. The body portion 401 comprises side walls and a bottom wall. The tray 400 may be formed by press-forming, thermo-forming or vacuum-forming.

The tray 300, 400 may for example be covered with a film, such as an optionally transparent plastic film, to protect the contents of the tray 300, 400, such as food. Such a film is preferably releasably adhered to the rim portion 302, 402 of the tray 300, 400.

Fig 5 shows an embodiment of a clamshell package 500 formed in a coated paper material according to the present disclosure. The paper substrate is composed of FibreForm®. A coated side of the material is printed. The clamshell package 500 comprises a generally bowl-shaped base portion 501 hingedly connected to a generally bowl-shaped top portion 502. Thus, the clamshell package 500 may be closed by folding along a hinging fold line 503. The base portion 501 comprises a generally flat bottom 504 and the top portion 502 comprises a decorative embossing 505 illustrating a flower. A substantially flat rim 506 of the base portion 501 is sealable against a substantially flat rim 507 of the top portion 502.

The stretchability of the paper substrate and the coating enables the bowl shapes of the bottom portion 501 and the top portion 502 as well as the decorative embossing 505 without significant impairment of the visual impression of the print. The clamshell package 500 may be formed by press-forming, thermo-forming or vacuum-forming. Vacuum forming or thermoforming normally requires that the paper material is provided with a gas barrier.

Fig 6 shows a base portion 601 of another embodiment of a clamshell package formed in a coated paper material according to the present disclosure. The paper substrate is composed of FibreForm®. A coated side of the material is printed. The base portion 601 is generally bowl-shaped and comprises a substantially flat rim 602 that is sealable against a corresponding rim of a top portion (not shown). The stretchability of the paper substrate and the coating enables allows the bowl shape to form without significant impairment of the visual impression of the print.

Fig 7 illustrates a sleeve 700 formed in a coated paper material according to the present disclosure. The paper substrate is composed of FibreForm®. An outer side of the sleeve is coated and printed. The sleeve 700 comprises a top wall 702, two opposing side walls 703 and a bottom wall. The sleeve 700 is arranged around a food-containing plastic package 701. A decorative/descriptive relief text ("FOOD") 704 has been formed in the upper wall 702 of the sleeve 200. The stretchability of the stretchable of the paper substrate and the coating allowed the relief text 704 to be formed in the top wall 702 without significant impairment of the visual impression of the print. The walls 702, 703 are joined by edges 705 defined by folding lines. The sleeve 700 is thus formed by folding and gluing a blank provided with folding lines.

Fig 8 illustrates a box 800 for a wine bottle. The box 800, which comprises four side walls 801, a top wall 802 and a bottom wall, is folded from a blank composed of a coated paper material according to the present disclosure. The paper substrate is composed of FibreForm®. The side of the material facing outwards is coated and printed. A decorative/descriptive relief 806 in the shape of a wine bottle has been formed in a side wall 801. The stretchability of the paper substrate and the coating allowed the relief 806 to be formed without significant impairment of the visual impression of the print. The box comprises four vertical edges 803, four horizontal edges 804 at the top and the four horizontal edges 805 at the bottom. At least three of the four vertical edges 803 are defined by folding lines made in the blank. Further, at least two of the four horizontal edges 804 at the top and at least two of the four horizontal edges 805 at the bottom are defined by folding lines made in the blank.

### EXPERIMENTAL SECTION

### Particle size distribution

In the experiments, the d₅₀ and *d*₉₈ values were measured using a Sedigraph 5120 from the company Micromeritics, USA. The method and the instrument are known to the skilled person and are commonly used to determine grain size of fillers and pigments. The measurements were carried out in an aqueous solution comprising 0.1 wt.-% Na₄P₂O₇. The samples were dispersed using a high speed stirrer and supersonics. For the measurement of dispersed samples, no further dispersing agents were added.

### Solids content of an aqueous suspension

The suspension solids content (also known as "dry weight") was determined using a Moisture Analyser MJ33 from the company Mettler-Toledo, Switzerland, with the following settings: drying temperature of 160°C, automatic switch off if the mass does not change more than 1 mg over a period of 30 s, standard drying of 5 to 20 g of suspension.

### Specific surface area (SSA)

The specific surface area was measured via the BET method according to ISO 9277 using nitrogen, following conditioning of the sample by heating at 250°C for a period of 30 minutes. Prior to such measurements, the sample is filtered within a Büchner funnel, rinsed with deionised water and dried overnight at 90 to 100°C in an oven. Subsequently the dry cake is ground thoroughly in a mortar and the resulting powder placed in a moisture balance at 130°C until a constant weight is reached.

### Fillers

In the experiments, three different fillers were used.
Filler 1: natural ground calcium carbonate; d₅₀ = 0.7 µm; *d*₉₈ = 5.0 µm; BET SSA = 11.5 m²/g; solids content 78 wt.-% (available from Omya, Switzerland)
Filler 2: natural ground calcium carbonate; d₅₀ = 1.5 µm; *d*₉₈ = 10.0 µm; BET SSA = 6.8 m²/g; solids content 78 wt.-% (available from Omya, Switzerland)
Filler 3: natural ground calcium carbonate; d₅₀ = 0.4 µm; *d*₉₈ = 2.0 µm; BET SSA = 18.0 m²/g; solids content 75 wt.-% (available from Omya, Switzerland)

### Coating preparation

In the experiments, different coating compositions were prepared and evaluated as described below. The respective filler slurries and binder slurries were combined in a beaker by gentle mixing resulting in coating compositions having initial solids contents. Subsequently, the aqueous coating compositions were mixed under higher shear conditions without drawing air until the individual phases of the composition were visually homogenously mixed. For adjustment of final solids contents of the aqueous coating compositions, calculated amounts of water were added by mixing again under higher shear conditions without drawing air. All mixing steps were done with a Pendraulik Laboratory Dissolver, model LD 50.

### Stretchabilitu testing method

To evaluate the stretchability of the compositions in the experiments, coating layers of the compositions were applied to a stretchable paper and tested with a newly developed 3D formability tester that was developed by Omya and built by Norbert Schläfli Maschinen (Zofingen). Schematic drawings indicating major dimensions of the formability tester built of aluminium are shown in Fig 9. The key element is a profiled wheel with a diameter of 125 mm and a width of 30 mm. The profile covers half of the circumference of the wheel, and develops like a membrane in bulge tests from a flat surface to a semi-circle. The stretch level develops continuously along the profile having a total testing length of 19.6 cm (wheel diameter * pi / 2) from 0% (30 mm stretching length and 30 mm stretched material) at the starting point to 57% (30 mm stretching length and 47.1 mm stretched material) at the end point. The wheel is part of an upper body of the testing instrument and is connected to two parallel rails that are also part of the upper body and guide the wheel when pulled manually for testing. The surface of the upper body that is showing towards the lower body is planar with the un-profiled section of the wheel. The lower body of the testing instrument is a massive block of aluminium with a 30 mm wide groove with broken edges not to cut the paper during testing when the profile is pressed into the paper. In order to avoid slipping paper during forming sandpaper can be glued just above the edge to firmly hold the testing paper between the upper and the lower body of the testing instrument.

For testing, coated paper is clamped between the upper and lower body of the testing instrument with the coated surface facing the groove of the lower body. Due to the fact that papers e.g. FibreForm® have a higher elongation at break in the machine direction (the direction the paper is produced, MD) the sample should be cut in the paper cross direction (CD) to use the higher stretchability in the MD, the wheel rolls in the CD and the stretch developed by the width of the wheel is applied in the MD, respectively. A trained person operates the testing instrument to ensure comparable results with regard to testing speed, clamping force and starting point of the measurement. The wheel rolls over the paper due to friction between paper and wheel surface and presses the profile into the paper. Obvious breaks of FibreForm® material without coating as described above have stretch levels of about 35-40% or brake after about 12 cm testing length. Coated samples were tested after 10 cm testing length or 29% of stretch.

To better visualize cracks, the coated surface is painted with Neocarmin W (MERCK), which is a testing liquid for colouring cellulose fibres that are visible at the cracks and gently cleaned with a soft tissue. Samples sufficiently large for microscopic evaluation are cut from the middle of the test area at a testing length of 10 cm and glued to a flat carton board. A stereo microscope is used to image the sample (Leica) at about 16 times magnification.

These images can be used for qualitative evaluation or further analysed by image analysis means.

### Application and testing of coating compositions

In the experiments, the coatings were applied to the substrate with a variable speed drawdown coater (K Control Coater 303 Model 625 available from Erichsen GmbH & Co. KG, Hemer, Gemany; 12 speed steps increasing from 2 and 40m/min and 10 application rods allowing increasing application weights at given speeds).

The coated samples were stretched in the 3D formability tester as described above.

Subsequently, the formation of cracks was investigated by the evaluation of microscopic images.

### Binder type screening

A general screening was carried out to identify a suitable type of binder. In the screening, coating compositions comprising 100 parts (dry weight) of Filler 1 and 20 parts (dry weight) of various binders were prepared and applied to a stretchable paper substrate (100 g/m² FibreForm® (BillerudKorsnäs) (not a laminate)). The solids content of the compositions was about 60 %. Coating was carried out in the machine direction and the coat weight was about 20 g/m². Sample strips were cut from the coated substrate. A textile color (Neocarmin) was applied to visualize cracks. The strips were stretched and microscopic images were taken. The images were then analyzed. The results are presented in the table 1 below.

**Table 1. "SA" refers to styrene-acrylic copolymer and "VA" refers to vinyl-acrylic copolymer.**

| Trade name | Type | Tg (°C) | Solids content (%) | Coat weight (g/m²) | Cracking |
|---|---|---|---|---|---|
| Appretan E2100 | Pure acrylic | -30 | 61.4 | 20.2 | Acceptable |
| Appretan E6200 | SA | -20 | 61.5 | 20.6 | Acceptable |
| Appretan E4250 | VA | -15 | 61.5 | 19.4 | Acceptable |
| Primal 325 GB | SA | -25 | 60.8 | 20.5 | Acceptable |
| Primal P-308 MS | SA | 8 | 61.5 | 20.2 | Unacceptable |

As can be seen in table 2, all binders giving an acceptable degree of cracking had a Tg below 8 °C.

### Binder level

Tests were carried out to find an appropriate level/amount of binder. In the tests, coating compositions comprising 100 parts (dry weight) of Filler 1 and 10, 15 or 20 parts (dry weight) of the binder Appretan E2100 were prepared and applied to a stretchable paper substrate (100 g/m² FibreForm® (Billerudkorsnäs) (not a laminate)). The solids content of the compositions was about 60 %. Coating was carried out in the machine direction and the coat weight was about 20 g/m². Sample strips were cut from the coated substrate. A textile color (Neocarmin) was applied to visualize cracks. The strips were stretched and microscopic images were taken. The images were then analyzed and the cracking in each coating was quantified. A "cracking number" was assigned to each composition. The results are presented in the table 2 below.

**Table 2.**

| Binder | Filler | Solids content (%) | Coat weight (g/m²) | Cracking |
|---|---|---|---|---|
| 10 parts | 100 parts | 63.0 | 19.5 | 104k, Unacceptable |
| 15 parts | 100 parts | 63.1 | 20.2 | 63k, Acceptable |
| 20 parts | 100 parts | 62.0 | 61.4 | 48k, Acceptable |

From table 2, it is concluded that at least 15 parts of binder is needed for an acceptable result. It is further concluded that more than 15 parts, such as at least 16 parts, is preferred as 20 parts resulted in less cracking than 15 parts.

### Pigment particle size

Tests were carried out to find an appropriate pigment particle size. In the tests, coating compositions comprising 100 parts (dry weight) of inorganic filler and 20 parts (dry weight) of the binder Appretan E2100 were prepared and applied to a stretchable paper substrate (100 g/m² FibreForm® (Billerudkorsnäs) (not a laminate)). Three different inorganic fillers having different particle sizes were tested. The solids content of the compositions was about 60 %. Coating was carried out in the machine direction and the coat weight was about 20 g/m². Sample strips were cut from the coated substrate. A textile color (Neocarmin) was applied to visualize cracks. The strips were stretched and microscopic images were taken. The images were then analyzed and the cracking in each coating was quantified. A cracking number was assigned to each composition. The results are presented in the table 3 below.

**Table 3. "BET SSA" refers to BET specific surface area.**

| Filler | BET SSA (m²/g) | *d₉₈* (µm) | *d₅₀* (µm) | Solids content (%) | Coat weight (g/m²) | Cracking |
|---|---|---|---|---|---|---|
| Filler 2 | 6.8 | 10 | 1.4 | 63.2 | 19.0 | 29k, Acceptable |
| Filler 1 | 11.5 | 5 | 0.7 | 61.4 | 19.1 | 48k, Acceptable |
| Filler 3 | 18 | 2 | 0.5 | 56.8 | 19.2 | 64k, Acceptable |

As can be seen in table 3, all three types of fillers tested resulted in acceptable cracking. It is however concluded from table 3 that it is preferred to use a filler having a BET specific surface area of less than 18 m²/g as Filler 1 and 2 resulted in substantially less cracking than Filler 3.

### Paper surface properties

Printing properties of coating compositions according to the present disclosure as well as changes in the print quality after paper 3D-forming were investigated by a continuous lab-scale coating and printing trial.

The coating compositions comprised 100 parts (dry weight) of Filler 1 and 15 parts (dry weight) of one of three different binders (see table 4). The coating compositions were applied to a stretchable paper substrate (100 g/m² FibreForm® (Billerudkorsnäs) (not a laminate)) with a Durrer continuous lab coating machine, using rod metering (C23, rod pressure of about 1 bar, rod revolution 12 rpm) at a coating speed of 20 m/min.

Coated paper surface properties were evaluated with regard to optical properties (CIE whiteness) and smoothness (Parker Print Surfaces).

3D-forming tests of the coated sheets were done as described above.

**Table 4.**

| Trade name (binder) | Type | Tg (°C) | Solids content (%) | Coat weight (g/m²) |
|---|---|---|---|---|
| Appretan E2100 | Pure acrylic | -30 | 58.3 | 19.5 |
| Appretan E6200 | SA | -20 | 58.7 | 19.0 |
| Primal 325 GB | SA | -25 | 58.1 | 18.0 |

As expected, coating compositions of table 4 significantly improved the paper surface quality in terms of whiteness and smoothness. 3D-forming resulted in some tiny (but acceptable) cracks in the coating layers, which indicated that 15 parts is at the lower end of acceptable binder levels.

## Claims

1. A coated paper material comprising a paper substrate coated with a composition comprising:
at least one polymeric binder having a glass transition temperature (Tg) of -3 °C or lower, and
at least one inorganic filler having a BET specific surface area in the range of 2.0 to 20.0 m²/g,
wherein the dry weight ratio of the at least one polymeric binder to the at least one inorganic filler is between 15:100 and 20:100, such as between 16:100 and 20:100 and
wherein the at least one polymeric binder is at least one acrylic binder and
wherein the at least one polymeric binder and the at least one inorganic filler together constitute at least 90 wt.-% of the composition, based on the dry weight of the composition.

2. The coated paper material according to claim 1, wherein the paper substrate comprises at least two paper layers including a top paper layer that is coated with the composition.

3. The coated paper material according to claim 1 or 2, wherein the stretchability (ISO 1924/3) of the paper substrate or the top paper layer thereof is at least 3 %, such as at least 5 % or 7%, in the machine direction (MD) and/or the cross direction (CD).

4. The coated paper material according to any one of the preceding claims, wherein the Tg of the at least one polymeric binder is -10 °C or lower, such as -15 °C or lower, such as -20 °C or lower.

5. The coated paper material according to any one of the preceding claims, wherein the BET specific surface area of the at least one inorganic filler is in the range of 3.0 to 17.5 m²/g, such as 4.0 to 15 m²/g, such as 5.0 to 13 m²/g.

6. The coated paper material according to any one of the preceding claims, wherein the at least one polymeric binder is selected from the group consisting of:
acrylic homopolymers;
methacrylic homopolymers;
copolymers composed of at least two different monomers, one monomer having an acrylic or methacrylic functional group and the other monomer having a functional group selected from the group consisting of styrene, vinyl and allyl; and
mixtures thereof.

7. The coated paper material according to any one of the preceding claims, wherein the at least one polymeric binder is an acrylic homopolymer, a vinyl-acrylic copolymer, a styrene-acrylic copolymer, or a mixture thereof.

8. The coated paper material according to any one of the preceding claims, wherein the weight median particle size *d₅₀* of the at least one inorganic filler is in the range of 0.1 to 5.0 µm, such as 0.3 to 3.0 µm, such as 0.4 to 2.0 µm, such as 0.5 to 1.5 µm.

9. The coated paper material according to any one of the preceding claims, wherein the at least one inorganic filler is selected from the group consisting of calcium carbonate containing material, clay, kaolin and mixtures thereof, wherein calcium carbonate containing material is selected from the group consisting of natural ground calcium carbonate (GCC), precipitated calcium carbonate (PCC), dolomite and mixtures thereof.

10. The coated paper material according to any one of the preceding claims, wherein a coated surface of the coated paper material is printed, which printed surface is optionally covered by a barrier layer.

11. A package comprising at least one wall composed of the coated paper material according to any one of claims 1-10.

12. The coated paper material or package according to any one of claim 1-10 comprising a bulge or relief formed by stretching a portion of the coated paper material.

13. A method of forming a three-dimensional pattern comprising a step of subjecting an article comprising a coated paper material according to any one of claims 1-10 to a forming operation, such as press-forming or thermo-forming, to form the three-dimensional pattern in the coated paper material, wherein part of the coated paper material is stretched during the forming operation.

## Patentansprüche

1. Beschichtetes Papiermaterial, umfassend ein Papiersubstrat, das mit einer Zusammensetzung beschichtet ist, die Folgendes umfasst:
mindestens ein polymeres Bindemittel mit einer Glasübergangstemperatur (Tg) von -3 °C oder weniger und mindestens einen anorganischen Füllstoff mit einer BETspezifischen Oberfläche im Bereich von 2,0 bis 20,0 m²/g,
wobei das Trockengewichtsverhältnis des mindestens einen polymeren Bindemittels zu dem mindestens einen anorganischen Füllstoff zwischen 15:100 und 20:100 liegt, z. B. zwischen 16:100 und 20:100, und
wobei es sich bei dem mindestens einen polymeren Bindemittel um mindestens ein Acryl-Bindemittel handelt und wobei das mindestens eine polymere Bindemittel und der mindestens eine anorganische Füllstoff zusammen mindestens 90 Gew.-% der Zusammensetzung ausmachen, basierend auf dem Trockengewicht der Zusammensetzung.

2. Beschichtetes Papiermaterial nach Anspruch 1, wobei das Papiersubstrat mindestens zwei Papierschichten umfasst, die eine obere Papierschicht umfassen, welche mit der Zusammensetzung beschichtet ist.

3. Beschichtetes Papiermaterial nach Anspruch 1 oder 2, wobei die Dehnbarkeit (ISO 1924/3) des Papiersubstrats oder der oberen Papierschicht davon in der Maschinenrichtung (MD) und/oder in der Querrichtung (CD) mindestens 3 % beträgt, z. B. mindestens 5 % oder 7 %.

4. Beschichtetes Papiermaterial nach einem der vorhergehenden Ansprüche, wobei die Tg des mindestens einen polymeren Bindemittels -10 °C oder weniger beträgt, z. B. -15 °C oder weniger, z. B. -20 °C oder weniger.

5. Beschichtetes Papiermaterial nach einem der vorhergehenden Ansprüche, wobei die BET-spezifische Oberfläche des mindestens einen anorganischen Füllstoffs im Bereich von 3,0 bis 17,5 m²/g liegt, z. B. bei 4,0 bis 15 m²/g, z. B. bei 5,0 bis 13 m²/g.

6. Beschichtetes Papiermaterial nach einem der vorhergehenden Ansprüche, wobei das mindestens eine polymere Bindemittel ausgewählt ist aus der Gruppe bestehend aus:
Acryl-Homopolymeren;
Methacryl-Homopolymeren;
Copolymeren, die aus mindestens zwei verschiedenen Monomeren zusammengesetzt sind, wobei ein Monomer eine funktionelle Acryl- oder Methacrylgruppe aufweist und das andere Monomer eine funktionelle Gruppe ausgewählt aus der Gruppe bestehend aus Styrol, Vinyl und Allyl aufweist; und
Mischungen davon.

7. Beschichtetes Papiermaterial nach einem der vorhergehenden Ansprüche, wobei es sich bei dem mindestens einen polymeren Bindemittel um ein Acryl-Homopolymer, ein Vinyl-Acryl-Copolymer, ein Styrol-Acryl-Copolymer oder eine Mischung davon handelt.

8. Beschichtetes Papiermaterial nach einem der vorhergehenden Ansprüche, wobei die gewichtete mediane Teilchengröße *d₅₀* des mindestens einen anorganischen Füllstoffs im Bereich von 0,1 bis 5,0 µm liegt, z. B. bei 0,4 bis 2,0 µm, z. B. bei 0,5 bis 1,5 µm.

9. Beschichtetes Papiermaterial nach einem der vorhergehenden Ansprüche, wobei der mindestens eine anorganische Füllstoff ausgewählt ist aus der Gruppe, bestehend aus Calciumcarbonat enthaltendem Material, Ton, Kaolin und Mischungen davon, wobei das Calciumcarbonat enthaltende Material aus der Gruppe bestehend aus natürlichem gemahlenem Calciumcarbonat (GCC), gefälltem Calciumcarbonat (PCC), Dolomit und Mischungen davon ausgewählt ist.

10. Beschichtetes Papiermaterial nach einem der vorhergehenden Ansprüche, wobei eine beschichtete Fläche des beschichteten Papiermaterials bedruckt ist, wobei die bedruckte Fläche gegebenenfalls von einer Sperrschicht bedeckt ist.

11. Verpackung, umfassend mindestens eine Wand, die aus dem beschichteten Papiermaterial nach einem der Ansprüche 1 bis 10 zusammengesetzt ist.

12. Beschichtetes Papiermaterial oder Verpackung nach einem der Ansprüche 1 bis 10, umfassend eine Ausbuchtung oder ein Relief, die bzw. das durch Dehnen eines Teils des beschichteten Papiermaterials geformt wird.

13. Verfahren zum Formen eines dreidimensionalen Musters, umfassend einen Schritt des Unterziehens eines Gegenstandes, der ein beschichtetes Papiermaterial nach einem der Ansprüche 1 bis 10 umfasst, einem Formungsvorgang, wie z. B. Pressformen oder Thermoformen, um das dimensionale Muster in dem beschichteten Papiermaterial zu formen, wobei ein Teil des beschichteten Papiermaterials während des Formungsvorgangs gedehnt wird.

## Revendications

1. Matériau de papier enduit un substrat de papier enduit d'une composition comprenant :
au moins un liant polymérique possédant une température de transition du verre (Tg) inférieure à - 3° C, et
au moins une charge inorganique possédant une zone de surface spécifique BET comprise dans la gamme allant de 2,0 à 20,0 m²/g,
dans lequel le rapport du poids sec de l'au moins un liant polymérique à l'au moins une charge inorganique est compris entre 15:100 et 20:100, tel qu'entre 16:100 et 20:100 et
dans lequel au moins un liant polymérique est au moins un liant acrylique et
dans lequel au moins un liant polymérique et l'au moins une charge inorganique ensemble constituent au moins 90 % en poids de la composition, sur la base du poids sec de la composition.

2. Matériau de papier enduit selon la revendication 1, dans lequel le substrat de papier comprend au moins deux couches de papier y compris une couche de papier supérieur qui est enduite avec la composition.

3. Matériau de papier enduit selon la revendication 1 ou la revendication 2, dans lequel l'étirabilité (ISO 1924/3) du substrat de papier ou de la couche de papier supérieure de celui-ci est d'au moins 3 %, telle qu'au moins 5 % ou 7 %, dans la direction de machine (MD) et/ou dans la direction transversale (CD).

4. Matériau de papier enduit selon l'une quelconque des revendications précédentes, dans lequel la Tg de l'au moins un liant polymérique est inférieure à -10° C, telle qu'inférieure à -15° C, telle qu'inférieure à -20° C.

5. Matériau de papier enduit selon l'une quelconque des revendications précédentes, dans lequel la zone de surface spécifique BET de l'au moins une charge inorganique est comprise dans la gamme allant de 3,0 à 17,5 m²/g, telle que comprise entre 4,0 et 15 m²/g, telle que comprise entre 5,0 et 13 m²/g.

6. Matériau de papier enduit selon l'une quelconque des revendications précédentes, dans lequel l'au moins un liant polymérique est choisi parmi le groupe constitué :
d'homopolymères acryliques ;
d'homopolymères méthacryliques ;
de copolymères composés d'au moins deux différends monomère, un monomère possédant un groupe fonctionnel acrylique ou méthacrylique et l'autre monomère possédant un groupe fonctionnel choisi parmi le groupe constitué du styrène, du vinyle et de l'allyle ; et
de mélanges de ceux-ci.

7. Matériau de papier enduit selon l'une quelconque des revendications précédentes, dans lequel l'au moins un liant polymérique est un homopolymère acrylique, un copolymère vinyle-acrylique, un copolymère styrène-acrylique, ou un mélange de ceux-ci.

8. Matériau de papier enduit selon l'une quelconque des revendications précédentes, dans lequel la taille de particule moyenne en poids d50 de l'au moins une charge inorganique est comprise dans la gamme allant de 0,1 et 5,0 µm, telle que comprise entre 0,3 et 3,0 µm, telle que comprise entre 0,4 et 2,0 µm, telle que comprise entre 0,5 et 1,5 µm.

9. Matériau de papier enduit selon l'une quelconque des revendications précédentes, dans lequel l'au moins une charge organique est choisie parmi le groupe constitué d'un matériau contenant du carbonate de calcium, de l'argile, du kaolin et des mélanges de ceux-ci, dans lequel le matériau contenant du carbonate de calcium est choisi parmi le groupe constitué du carbonate de calcium naturel broyé (GCC), du carbonate de calcium précipité (PCC), de la dolomite et des mélanges de ceux-ci.

10. Matériau de papier enduit selon l'une quelconque des revendications précédentes, dans lequel une surface enduite du matériau de papier enduit est imprimée, dont la surface imprimée est éventuellement recouverte d'une couche barrière.

11. Paquet comprenant au moins une paroi composée du matériau de papier enduit selon l'une quelconque des revendications 1 à 10.

12. Matériau de papier enduit ou paquet selon l'une quelconque des revendications 1 à 10 comprenant une bosse ou un relief formé par l'étirage d'une partie du matériau de papier enduit.

13. Procédé de formation d'un motif à trois dimensions comprenant une étape consistant à soumettre un article comprenant un matériau de papier enduit selon l'une quelconque des revendications 1 à 10 à une opération de formation, telle qu'un procédé de formation sous pression ou de formation par la chaleur, pour former le motif à trois dimensions dans le matériau de papier enduit, dans lequel une partie du matériau de papier enduit est étirée pendant l'opération de formation.
